

# UNITED STATES PATENT OFFICE.

EDMUND R. BULLOCK, OF ROCHESTER, NEW YORK, ASSIGNOR TO EASTMAN KODAK COMPANY, OF ROCHESTER, NEW YORK, A CORPORATION OF NEW YORK.

## TELLURIUM TONING-BATH AND PROCESS OF TONING PHOTOGRAPHIC ELEMENTS.

1,273,797.

No Drawing.

Specification of Letters Patent.

Patented July 23, 1918.

Application filed April 5, 1916. Serial No. 89,017.

To all whom it may concern:

Be it known that I, EDMUND R. BULLOCK, of Rochester, county of Monroe, State of New York, have invented certain new and useful Improvements in Tellurium Toning-Baths and Processes for Toning Photographic Elements; and I do hereby declare the following to be a full, clear, and exact description of the same.

- 10 My invention relates to photography and more particularly to toning baths and the process of toning photographic prints and has for its object the provision of a satisfactory and easily manipulated toning bath 15 and a process for toning whereby a rich brown or sepia color effect may be obtained which is highly pleasing to the eye. To this and other ends, as will appear from the following disclosure, my invention resides in 20 the combination of parts and the steps of the process as set forth in the appended claims.

In the practice of my invention, I utilize a toning bath for transforming the ordinary 25 black and white tones of a silver image into a brown or sepia color effect which comprises an acid solution containing a compound of tellurium and which furnishes a molecular compound or an ion in solution 30 capable of reacting with silver to form an image which is insoluble in water or preferably insoluble in the toning bath.

A solution of a tellurium halid, preferably a chlorid of tetravalent tellurium, in 35 a hydrogen halid acid is found to be well suited for this purpose and to produce excellent sepia tones. While an excess of acid in the solution is preferred, there should be utilized sufficient acid to oppose any tendency 40 toward complete hydrolysis and maintain some tellurium salt in solution to carry on the toning reaction. A bath involving the halid of tellurium may be formed, for example, by dissolving tellurium dioxid 45 ( $\text{TeO}_2$ ) in hydrochloric acid, an excess of the latter being present. The tetravalent tellurium salt, tellurium chlorid ( $\text{TeCl}_4$ ), is probably present in the bath and serves as the reagent which forms with the silver 50 image a compound that is substantially insoluble in the toning bath.

If an ordinary photographic print or other element, such as plate, film or paper bearing a silver image which has been developed, fixed and washed in the usual man-

ner, is immersed in the tellurium bath, the photographic print or other element changes from its former approximately black or silver color to a sepia tone, probably due to the formation of a compound of silver and tellurium according to the following equa- 60



in which "X" represents the halogen or 65 other ion that reacts with the silver to form the insoluble compound. Both the resultant products in the above reaction are insoluble in the bath, but the silver-tellurium compound due to its predominating color 70 furnishes the tone to the image, the other salt merely degrading the color effect somewhat.

Since the bath should be free from injurious substances or those which tend to attack 75 the gelatin too strongly or which have a tendency to dissolve the silver before it has had time to tone, or to dissolve the silver-tellurium compound after the toning has taken place, I preferably utilize dilute 80 hydrochloric acid as the solvent for the tellurium compound. However, due to the slowness of reaction of the tellurium chlorid in hydrochloric acid on the silver image, I find it desirable that the bath contain an additional agent to accelerate the velocity of 85 the toning process. Also, it is found that after the toning has taken place and the print is being washed, the extreme dilution of the solution of the tellurium compound 90 present in the pores of the gelatin tends to form a precipitate of the oxid or hydrated oxid on the print, although acid has been used in the initial solution. This deposit, at first white in color, tends to be gradually reduced 95 by the gelatin to form a black deposit over the entire print. To overcome the formation of an undesirable precipitant and to accelerate the reaction velocity, I add to the tellurium halid bath a halid of an alkali 100 metal, preferably a bromid. Advantageous results are obtained by using a mixture of sodium chlorid and potassium bromid. By utilizing these salts it is possible to dilute the toning bath indefinitely or to wash the 105 print completely without danger of precipitation of an undesirable tellurium compound because of hydrolysis.

As a specific example, the following ingredients and proportion measured in grams 110

and cubic centimeters may be employed for use with one well known brand of photographic silver emulsion paper, although, of course, they may be varied to accord with the character of any other kind of photographic element that is to be sepia toned:

10      4 gm.  $\text{TeO}_2$ .  
         9 cc. HCl (concentrated.)  
         9 gm. NaCl.  
          $\frac{1}{2}$  gm. KBr.  
         Water to make 100 cc.

While the chemical structure of the compounds present in the tellurium bath and the exact nature of their reactions is immaterial, so far as the character and operation of my invention is concerned, there may possibly be present in the acid bath containing the alkali metal halid salts, a double salt of the type  $\text{Na}_2\text{TeBr}_6$ ; however, the reaction may be represented as proceeding according to the following simple formula, tellurium chlorid being considered the reactive agent:



By using baths of the above specific natures, a sepia tone is obtained, no further chemical treatment of the print being necessary. However, it is preferable to add another step to the process to obtain a deeper and richer effect and to regain the density of the original print, which was slightly reduced by the bleaching action of the tellurium bath. I, accordingly, wash the print, preferably in running water, for a sufficient time to remove the acid solution and then treat the image with a  $\text{Na}_2\text{S}$  solution, preferably a two per cent. solution of sodium sulfid crystals. The result of this step is probably to transform the white or light colored silver bromid or silver chlorid, which otherwise would tend to change to a 45 photobromid or photochlorid upon exposure of the photographic element to light, into the dark colored and more permanent silver sulfid, the print being given thereby substantially the same density as was originally 50 present.

The operation of my process is simple. An ordinary silver print, for example, after the usual developing, fixing and washing operations, is immersed in a tray containing 55 my tellurium toning bath or otherwise treated therewith for about two minutes or until the visible change in the print is complete, preferably while the tray is rocked or the solution otherwise stirred. It is inadvisable 60 to prolong the treatment of the print with the tellurium solution after a satisfactory result is obtained, as the color values may be disadvantageously affected thereby. The print may then be washed and dried, or, if 65 the sodium sulfid treatment is desired, it is

washed preferably until the acid has been substantially eliminated and then treated with a two per cent. aqueous solution of sodium sulfid to darken and intensify the print. When the color change has taken 70 place, the print is washed and dried in the usual manner to complete the process.

Having described my invention, I claim:

1. A photographic toning bath for silver images comprising a tellurium compound in 75 an acid solution, said bath being capable of converting the silver image into one which is insoluble therein.

2. A photographic toning solution for silver images comprising a compound of tellurium and an acid, said solution being capable of forming a compound containing silver, tellurium, and a silver salt which are insoluble in said bath.

3. A photographic toning solution for silver images containing a compound of tetravalent tellurium and an acid, said solution comprising a substance which is capable of forming a compound containing silver, tellurium, and a silver salt that are insoluble in 90 said solution.

4. A photographic toning bath for silver images comprising a tellurium compound, water, and an acid which will prevent precipitation of a tellurium compound and will 95 not injuriously attack the silver image.

5. A photographic sepia toning bath comprising a tellurium salt in a solution containing a hydrogen halid acid.

6. A photographic sepia toning bath comprising a tellurium chlorid in a solution acidified only with hydrochloric acid.

7. A photographic toning bath comprising a solution containing a tellurium halid and an accelerating agent.

8. A photographic toning bath comprising a solution of a tellurium salt and an agent capable of retarding hydrolysis and precipitation of a tellurium compound upon dilution with water.

9. A photographic sepia toning bath comprising a tellurium chlorid in a solution containing hydrochloric acid in excess and a halid salt.

10. A photographic sepia toning bath comprising a tellurium compound in a solution containing hydrochloric acid in excess, sodium chlorid and potassium bromid.

11. A photographic toning bath comprising tellurium chlorid, hydrochloric acid in 120 excess, sodium chlorid and potassium bromid.

12. The process of sepia toning a photographic silver image comprising the step of treating the silver image with an acid solution containing a tellurium salt.

13. The process of toning a photographic silver image comprising the step of changing the color of the silver image by treating it with a solution of tellurium chlorid dis- 130

solved in an excess of hydrochloric acid and producing a silver compound that is insoluble in water.

14. The process of toning a photographic silver image comprising the steps of treating said image with a solution of a tellurium salt to produce a given tone and modifying said tone by treatment with a sulfid solution.

10 15. The process of toning a photographic silver image comprising the steps of treating the image with an acid solution of a tellurium salt to produce a given sepia tone and treating with sodium sulfid to modify 15 said tone.

16. The process of sepia toning a photographic silver image comprising the steps of bleaching and sepia toning the silver image with a solution containing a tellurium

halid and intensifying and modifying the 20 tone of the image by treating with a sodium sulfid solution.

17. The process of toning a photographic silver image comprising the steps of treating said image with an aqueous solution of 25 tellurium chlorid, hydrochloric acid, sodium chlorid and potassium bromid and thereby bleaching and toning the image, and intensifying and modifying the tone of the image by means of an aqueous sodium sulfid solu- 30 tion.

In witness whereof I affix my signature this 1st day of April, 1916 in the presence of two witnesses.

EDMUND R. BULLOCK.

Witnesses:

ALONZO S. McDANIEL,  
G. C. COOKE.